

Feb. 8, 1944.

D. TRAILL ET AL

2,340,909

MANUFACTURE OF ARTIFICIAL FIBERS FROM PROTEIN MATERIAL

Filed Dec. 7, 1939



FIG. 1.



FIG. 2.

Inventors

DAVID TRAILL  
ROBERT V. SEDDON  
WILLIAM SEVER

By

*A. M. Young, Jr.*  
their Attorney

## UNITED STATES PATENT OFFICE

2,340,909

MANUFACTURE OF ARTIFICIAL FIBERS  
FROM PROTEIN MATERIAL

David Traill, Ardrossan, Robert Vincent Seddon,  
Salteats, and William Sever, Troon, Scotland,  
assignors to Imperial Chemical Industries Limited,  
a corporation of Great Britain

Application December 7, 1939, Serial No. 308,102  
In Great Britain January 21, 1939

11 Claims. (Cl. 18--54)

The present invention relates to the manufacture of artificial fibers from the vegetable globulins separable from ground-nuts or peanuts (*Arachis hypogaea*); that is, the globulins known as arachins. The invention may be applied either in the manufacture of fibers suitable for use in the manufacture of brushes and the like, which fibers will be referred to hereinafter as bristles; or in the manufacture of finer textile filaments having some of the properties of wool and silk. The fibers of the present invention do not possess the organised structure of the hair of animals; but they can be used, either alone or in association with other fibers, in the manufacture of brushes, textile fabrics, or the like; and in their chemical and physical properties they resemble animal hair more closely than filaments or fibers of cellulosic origin.

In certain recent inventions textile fibers of a character like that of wool are produced from the globulins of the peanut or ground-nut (*Arachis hypogaea*); the arachins. The ground-nut protein is usually extracted from ground-nut meal (from which the oil has ordinarily been removed) at ordinary temperatures with dilute aqueous alkaline or saline solutions, and is precipitated by addition of a suitable quantity of acid.

The dry recovered globulin is taken up in urea solution, giving a dispersion which is at first liquid enough to permit clarification but afterwards thickens to a consistency enabling its extrusion from the ordinary spinnerets used in making other artificial fibers. These ordinary spinnerets have a very fine bore; that appropriate for making a textile fiber. In the prior processes the extruded filaments are treated by various processes to give them a flexible thread-like character.

We have now found that these globulins can be dispersed in another way, giving liquids with which the viscosity can be adjusted; giving not only liquids adapted for extrusion from these fine spinnerets to produce textile fibers but also from spinnerets of coarser bore to give bristle-like extrusion. By appropriate treatment the thicker extrusions can be given bristle characteristics.

When ground-nut protein thus isolated is taken up in aqueous ammonia it disperses to form what may appear to be a solution, but if the protein concentration is sufficient the liquid reveals a pasty character. The untreated ammoniacal apparent solutions of ground-nut protein cannot be used for the production of fibers by extrusion through nozzles and treatment in coagulating baths with or without tension on the

extruded fiber. They are referred to hereinafter as crude ammoniacal dispersions.

We have found that when these crude ammoniacal dispersions of ground-nut protein are subjected to thermal treatment at a temperature not below about 60° C. they undergo changes, the occurrence of which is marked by a considerable increase in their viscosity, which may be sufficient to lead to the gelation of the resulting viscous solution. We have further observed that the resulting viscous solutions or jellies are strongly thixotropic in character and that fibers of either bristle or filamentary character can be obtained from them by extrusion into coagulating baths.

According to the present invention, fibers are obtained by the extrusion, into a coagulating bath, of a thixotropic viscous solution made by a thermal treatment that comprises maintaining at a temperature not below about 60° C. a crude dispersion of ground-nut protein in dilute aqueous ammonia until an increase in natural viscosity at least of the order of 5-fold as determined in the manner hereinafter described has been obtained, and if necessary applying a mechanical shearing treatment to the resulting hot viscous solution or jelly sufficient to bring about a desired reduction in viscosity, prior to extrusion. The increase in the natural viscosity is determined by comparing at similar atmospheric temperatures the viscosity of the original dispersion and that of the material obtained from it by conducting both the thermal treatment and the subsequent cooling in the absence of any mechanical shearing treatment.

For the purpose of observing the viscosity of the original ammoniacal dispersion a sufficient time should be allowed to elapse between the making up of the dispersion and the measurement of its viscosity in order to allow the latter to reach an approximately steady value corresponding to the completion of the dispersion process. If desired this may be hastened by mechanically homogenising the mixture, or by warming it to some temperature well below that at which the said changes occur.

A suitable ground-nut protein concentration is from about 10 to about 25 per cent and the aqueous ammonia used is suitably between 0.2 and 2 per cent ammonia concentration, and advantageously from 0.5 to 1 per cent.

The time for which it is necessary to heat the aqueous ammoniacal protein dispersion in order to bring about the desired changes decreases in a very high degree as the temperature is increased.

but the thermal treatment of a given dispersion may advantageously be carried out until it has attained the same viscosity as it attains after 2½ to 3 hours heating at 70° C. under otherwise similar conditions.

The temperature at which it is most desirable to extrude the viscous solution may be different from the temperature at which the thermal treatment is carried out. If the natural viscosity of the product obtained by the thermal treatment is too high to permit of its use at the desired spinning temperature, as for instance, when it has gelated, the viscous solution or jelly is subjected to a mechanical shearing treatment. By this means its viscosity may be thixotropically reduced to a convenient value and if necessary it is maintained in motion until it is to be employed. For carrying out the mechanical shearing treatment, many types of apparatus may be used but colloid mills, homogenisers, and emulsifiers are particularly useful.

For the production of filaments it is especially desirable that the protein concentration should be sufficiently high for the thermal treatment to yield a more or less gelated product if a mechanical shearing treatment is omitted; and advantageously not less than 20 parts by weight of the protein are used to each hundred parts by weight of aqueous ammonia.

When the concentration of the protein is such that the thermal treatment of the aqueous ammoniacal dispersion when carried out without any mechanical shearing treatment yields more or less gelated products, it is often desirable to commence the mechanical shearing treatment that is required for the reduction of the viscosity while the thermal treatment is actually being carried out, because although the natural rise in viscosity is thereby partly checked and gelation is prevented, the desirable effect of the thermal treatment in rendering the protein capable of being made into fibers is not unfavourably influenced. By this method a homogeneous solution free from air bubbles is more easily obtained than when the gelation has been allowed to take place before the mechanical shearing treatment is commenced.

Suitable coagulating baths for the production of fibers according to our invention include, for instance, acid solutions and acidified saline solutions, for instance aqueous solutions of sulphuric acid with or without sodium or ammonium sulphate, but other coagulating baths known in the art of making fibers may also be used. In making fibers, the protein solution as above prepared is extruded into the coagulating bath. The fibers produced according to our invention should be subjected to an after-treatment with formaldehyde or other hardening agent, and are advantageously also subjected to a treatment with substances adapted to yield non-ionized HCl, to increase their resistance to wet processing, for instance as described in British Patents Nos. 492,895, 492,677 and 495,332, or British application No. 8659/38 (corresponding to the U. S. application Serial No. 263,094 of Fieldsend and Boyes, filed March 20, 1939).

The invention is further illustrated by the following examples in which the parts mentioned are parts by weight; and by the accompanying drawing, in which

Fig. 1 is a schematic view illustrative of an apparatus organization useful in performing the process of Example 1 and

Fig. 2 is a schematic showing of apparatus useful in performing the process of Example 3.

The drawing will be described in reference to the examples.

5

### Example 1

This example illustrates the manufacture of an artificial bristle.

Forty-four parts of ground nut protein prepared as described in British Patent No. 513,896 are ground to a paste with 100 parts of water, and another 135 parts of water are stirred in. Thereupon 30 parts of 5 per cent aqueous ammonia are added to the thin paste, and the mixture is passed through an emulsifier several times, whereby the dispersion is assisted. The dispersion is heated in a closed container at 70° C. for 2½ hours, and the resulting viscous solution is then allowed to cool to room temperature and to stand for 24 hours. Referring now to Fig. 1, the cooled solution is then extruded from a single-hole glass spinneret 5 having a bore of 1 mm. into a 30 per cent solution of sulphuric acid. The precipitated fiber 6, as shown, is drawn from the coagulating bath without tension at the rate of 1 metre per minute, and the length of its travel in the bath 7 is such that there is 1 minute's contact with the acid. The fiber is then passed through a bath 8 of 36 per cent aqueous formaldehyde over and under a number of rollers 9 of increasing diameter, so that it receives 10 minutes treatment and is stretched to one and one half times its original length. It is then washed in running water 10 for a period of 25 minutes until it is practically free from acid, and is drawn, still under tension, through a drying chamber 11 in counter-current to a stream of hot air, whereby it is partly dried, and the stretch is increased another 10 per cent. It is then wound on to a hexagonal swift 12, allowed to dry in straight lengths of about 5 to 6 inches, and cut to size. The bristles are then soaked in a 2 per cent solution of thionyl chloride in carbon tetrachloride at 35° C. for four days and are dried off.

45

### Example 2

A viscous solution is made from a ground-nut protein dispersion as described in Example 1 and is drawn under slight tension from a single-hole glass spinneret of the same diameter into 30 per cent sulphuric acid at the rate of 30 metres per minute, and is allowed to coil up in a vessel containing 30 per cent sulphuric acid, in which the coagulation is completed. The fiber is next drawn from the vessel at the rate of 1 metre per minute and hardened, washed, partly dried under tension, and further dried and cut as described in Example 1. The bristles are soaked for 24 hours at 35° C. in 50 times their weight of a solution containing 94.6 parts of saturated sodium chloride brine, 1.7 parts of 40 per cent formaldehyde and 3.7 parts of 35 per cent hydrochloric acid. They are then washed until free from salt and dried.

65

### Example 3

This example illustrates the manufacture of fine filaments according to the invention.

Twenty-three and one-half parts of ground-nut protein are stirred to a cream with 90 parts of water and 10 parts of 5 per cent aqueous ammonia. The mixture is first filtered to remove any hard particles and the dispersion is then transferred to a circulating apparatus comprising an open reservoir 15, a constant delivery pump 16, a tube or jet type of homogeniser 17, a

heating coil 18, and a manometer 19 attached to one of the necessary conduits leading to the open reservoir. The reservoir, the homogeniser and the coil portions of the apparatus are immersed in water baths 21, 22 and 23 respectively. The homogeniser serves both to make the initial dispersion as complete as possible and to control the viscosity of the viscous thixotropic solution into which the dispersion is gradually converted as the thermal treatment proceeds, so as to prevent the gelation of the product. The viscosity of the moving liquid is an approximately linear function of the pressure observed in the manometer since a constant rate of flow is maintained by the pump. In using the apparatus the dispersion is first circulated for one hour before any hot water is introduced into the water baths, and thus without raising its temperature. The water baths in which the homogeniser and the coil are immersed are then filled with water at 70-80° C. and the reservoir is heated to 60° by introducing hot water into its water bath. Circulation is continued for one hour, during which these temperatures are maintained. The viscosity at the circulation temperature first falls and then rises to 30 to 40 times the minimum value attained. The homogeniser, the coil, and the reservoir are then cooled and the solution is kept in continuous circulation until after some hours room temperature is attained and the viscosity measured during its motion becomes constant. The solution is then in spinnable condition but it must be maintained in continuous circulation until it is spun.

The solution so obtained is passed through a candle filter 20 and is extruded from a standard spinneret, not shown, having orifices of 0.08 mm. diameter, into a bath kept at 55° C. containing 35 parts of ammonium sulphate, 64 parts of water and 1 part of sulphuric acid, and wound at a rate of 80 metres of filament per minute. The size of the washed and dried filament is 3.5 denier. It is then subjected to after-treatment designed to improve its resistance to the action of water as described in the acknowledged British application 8659/38, or British Patents 495,332, 492,895 or 492,677.

The method of continuously passing the product during the thermal treatment to the apparatus for applying a mechanical shearing treatment and circulating it back again for further thermal treatment exemplified in Example 3 is of particular value in carrying out the present invention.

We claim:

1. A method of preparing ammoniacal dispersions or solutions of peanut protein of thixotropic character, as spinnable liquids of a viscosity enabling them to be extruded through orifices into coagulating baths to form fibers, which comprises subjecting a dispersion of peanut protein in amount 10 to 25 per cent in dilute aqueous ammonia of concentration approximately 0.2 to 2 per cent to a heat treatment in which the dispersion is kept at a temperature above approximately 60° C. until the viscosity of the dispersion, with reference to a sample thereof which is maintained in the absence of applied shearing stresses, is increased at least approximately five-fold with respect to that of the original dispersion.

2. A method of preparing ammoniacal dispersions or solutions of peanut protein of thixotropic character, as spinnable liquids of a viscosity enabling them to be extruded through orifices into coagulating baths to form fibers, which comprises

subjecting a dispersion of peanut protein in amount not less than about 20 per cent in dilute aqueous ammonia of concentration approximately 0.2 to 2 per cent, to a heat treatment in which the dispersion is kept at a temperature above approximately 60° C. until the viscosity of the dispersion, with reference to a sample thereof which is maintained in the absence of applied shearing stresses, is increased at least approximately five-fold with respect to that of the original dispersion.

3. The method of claim 1 wherein the dispersion is kept at a temperature of about 60° C. for 2.5 to 3 hours.

4. The method of claim 1 comprising, in addition, subjecting the dispersion to mechanical shearing stresses so as to reduce its viscosity.

5. The method of claim 1 comprising in addition the operation of subjecting the dispersion to mechanical shearing stresses during said thermal treatment.

6. A method of preparing ammoniacal dispersions or solutions of peanut protein of thixotropic character, as spinnable liquids of a viscosity enabling them to be extruded through orifices into coagulating baths to form fibers, which comprises subjecting a dispersion of peanut protein in amount 10 to 25 per cent in dilute aqueous ammonia of concentration approximately 0.2 to 2 per cent, to a heat treatment in which the dispersion is kept at a temperature above approximately 60° C. while continuously withdrawing portions of the dispersion, subjecting the withdrawn portions to mechanical shearing stresses and returning them to the heat treatment; and continuing said treatment until the viscosity of the dispersion, with reference to a sample thereof which is maintained in the absence of applied shearing stresses, is increased at least approximately five-fold with respect to that of the original dispersion.

7. The method of claim 1 comprising in addition the step of mechanically homogenizing the dispersion of peanut protein in ammonia, at a temperature below 60° C., preliminarily to said heat treatment.

8. In making artificial fibers from peanut protein, the process which comprises subjecting a dispersion of peanut protein in amount 10 to 25 per cent in dilute aqueous ammonia of concentration approximately 0.2 to 2 per cent to a heat treatment in which the dispersion is kept at a temperature above approximately 60° C. until the viscosity is increased at least approximately 5-fold, thereby forming a hot viscous thixotropic solution, extruding the solution without tension through a small orifice into a coagulating bath to form fibers, and hardening the extruded fibers in a formaldehyde bath under tension sufficient to produce extension to about 1.5 times the original length.

9. In methods of producing bristles from peanut protein which include the step of producing a dispersion of such protein in amount 10 to 25 per cent in dilute aqueous ammonia of concentration approximately 0.2 to 2 per cent, the improvement comprising thickening the dispersion by exposure to a temperature above 60° C. until a viscous thixotropic material is obtained, extruding the said viscous material through a small orifice into a coagulating bath and without tension, maintaining the extruded product in the coagulating bath for a length of time sufficient to coagulate the liquid and product a filament,

75 hardening the filament thus produced in a form-

aldehyde bath under tension for a longer period of time than was occupied in coagulation with the tension being sufficient to produce extension to 1.5 times the original length, washing and drying under tension.

10. The method of increasing the viscosity of ammoniacal dispersions of peanut protein to a point where they are thixotropic in character and of a viscosity suitable for extrusion by known extrusion procedures through orifices into coagulating baths to form fibers, which comprises heating a liquid dispersion of peanut protein in amount 10 to 25 per cent in dilute aqueous ammonia of concentration approximately 0.2 to 2 per cent at a temperature of about 70° C., withdrawing portions of the liquid dispersion from the main body thereof, subjecting the withdrawn portions to mechanical shearing stresses and re-

turning said withdrawn portions to the main body for further heating.

11. A method of preparing ammoniacal dispersions of peanut protein of thixotropic character and of viscosity suitable for fiber-forming by extrusion through small orifices into a coagulating bath, which comprises dispersing such protein in amount 10 to 25 per cent in dilute aqueous ammonia of concentration approximately 0.2 to 2 per cent and subjecting the dispersion to a thermal treatment at a temperature above 60° C., until its viscosity is increased to substantially the viscosity attained by heating an identical dispersion to a temperature of 70° C. for a period of 2½ to 3 hours.

DAVID TRAILL.  
ROBERT V. SEDDON.  
WILLIAM SEVER.